

## UNITED STATES PATENT OFFICE.

TRUMAN S. FULLER, OF SCHENECTADY, NEW YORK, ASSIGNOR TO GENERAL ELECTRIC COMPANY, A CORPORATION OF NEW YORK.

## RESISTANCE ALLOY.

No Drawing.

Application filed February 25, 1927. Serial No. 171,075.

- The present invention relates to alloys and more particularly to alloys employed in connection with electrical apparatus and commonly known as resistance alloys.
- 5 In the construction of dynamo electric machines of the induction type, it is common to form the conducting bars and end rings of the rotor member from cast aluminum. Pure aluminum bars and rings, however, 10 owing to their high degree of conductivity, are sometimes unsatisfactory for use in motors requiring a high starting torque, such, for example, as elevator motors and the like.
- 15 It is one of the objects of the present invention to provide a resistance alloy which has a higher resistance than aluminum but is suitable for use as conducting bars and end rings in induction motor rotors. Another 20 object of the invention is to provide a resistance alloy capable of being cast in a manner similar to aluminum and not greatly exceeding aluminum in cost of manufacture. A further object of the invention is to provide 25 a resistance alloy which may be held molten in air for a considerable period of time without suffering any appreciable change in its composition or conductivity.
- In carrying out my invention I provide 30 an alloy consisting mainly of aluminum but containing appreciable amounts of both manganese and zinc. Manganese and zinc each have a tendency to reduce the conductivity of aluminum although zinc has a 35 lesser tendency to do so than the manganese. The use of zinc in the alloy, however, in addition to reducing conductivity, provides an alloy which is not so brittle as that which might be obtained by a combination of alu- 40 minum and manganese alone and which has other desirable features as well. For example, an alloy having a content of about 92% aluminum and 8% manganese has a resistivity equal to about 11.5 microhms per centimeter cubed. Such an alloy, however, may 45 be found to be too brittle for certain uses. Addition of a small quantity of zinc to take the place of a portion of the manganese provides an alloy having the same degree of 50 resistivity but a lesser degree of brittleness than the aluminum-manganese alloy. The addition of zinc to the aluminum-manganese alloy also performs another valuable func-
- tion. The molten metal comprising the aluminum, manganese and zinc will usually 55 have a temperature of about 825°-850° C. when castings are made from the alloy, and it is often necessary to maintain a given quantity of the metal in a molten condition in air while the rotors of several machines 60 are cast. It is desirable, therefore, that the composition and resistance of the alloy should not change materially during this period. I have found that by the addition of a small percentage of zinc to a molten 65 alloy of aluminum and manganese, the resultant alloy remains substantially unchanged in composition while maintained at a temperature of 825°-850° C. for pro- 70 longed periods of time and that there is no change in the resistivity of several rotors which may be cast from any one melt.
- The zinc content of the alloy may range 75 from about 2 to 8% of the total content of the alloy, and the manganese from about 4 to 10% of the content of the alloy, the remainder of the alloy being aluminum. I have found that if the alloy consists of approximately 90% aluminum, 6% manganese and 4% zinc, uniformly satisfactory 80 results may be obtained. Such an alloy will not greatly exceed the cost of pure aluminum, will have a resistivity equal to about 11.5 microhms per centimeter cubed, and may be cast in a manner similar to 85 aluminum.
- What I claim as new and desire to secure by Letters Patent of the United States is:—
1. A resistance alloy consisting largely of aluminum and containing appreciable amounts of manganese and zinc. 90
  2. An alloy consisting largely of aluminum and containing from 4 to 10% of manganese and from 2 to 8% of zinc.
  3. An alloy consisting of about 90% alu- 95 minum, 6% manganese and 4% zinc.
  4. A resistance alloy consisting largely of aluminum and containing at least 4% manganese and having a resistance equal to about 11.5 microhms per centimeter cubed. 100
  5. A resistance alloy consisting largely of aluminum and containing at least 4% of manganese and at least 2% of zinc.
- In witness whereof, I have hereunto set my hand this 24th day of February, 1927.
- TRUMAN S. FULLER.